

April 28, 1964

B. BERGHAUS

3,130,671

METHOD OF REDUCING BARREL WEAR

Filed May 2, 1958



INVENTOR  
BERNHARD BERGHAUS

BY  
*Joseph Heischemann*  
ATTORNEY

3,130,671

## METHOD OF REDUCING BARREL WEAR

Bernhard Berghaus, Zurich, Switzerland, assignor to  
Elektrophysikalische Anstalt Bernhard Berghaus, Va-  
duz, Liechtenstein, a corporation of Liechtenstein

Filed May 2, 1958, Ser. No. 732,605

5 Claims. (Cl. 102—93)

The present invention relates to a method of reducing the wear of the inner barrel wall of firearms during the passage of projectiles, in particular in firearm barrels of which the inner wall has a surface layer enriched with a foreign substance.

The present invention is based on the generally known fact that firearm barrels are subject to a reduction in weight during firing, which is caused by the small quantity of liquid or vaporized barrel material ejected as each projectile is fired. Apparently the temperature at the points of the inner barrel wall subject to the greatest stress rises above the melting point during firing, at least in a thin surface layer, so that the inner wall melts at these points.

It seems natural for the resistance to wear of such firearm barrels to be increased by raising the melting point of the firearm barrels or at least of their inner wall. However, this is not possible as alloyed steels must be used for the barrel for reasons of strength while the surface zone of the inner wall is generally improved by enriching it with foreign substances, i.e. hardened by nitriding. Owing to the alloy components and the surface layer enriched with foreign substances, the melting point of the material of the inner wall is usually reduced.

The present invention has for its object to eliminate the drawbacks of this lowering of the melting point of the inner barrel wall in firearms of which a surface layer is enriched with foreign matter for other reasons. The method according to this invention of reducing the wear of the inner barrel wall of such firearms during the passage of a projectile is characterized by the fact that at least the driving bands of the projectile and at least their surface have the melting point of their material reduced at least substantially to the melting point of the inner barrel wall or provided with a lower melting point than the latter.

The invention also relates to a firearm and a projectile designed according to this method and characterized by the fact that at least the surface portions designed for contact and the adjacent deeper zones are enriched with materials of such kind that the projectile driving bands possess approximately the same or a lower melting point than the inner barrel wall under the prevailing pressure conditions.

The method is described in greater detail in conjunction with the attached drawing which illustrates an embodiment of the treatment of projectiles according to the present invention.

In present-day firearms the inner wall of the barrels is subject to very high stresses and it reaches a temperature, particularly in automatic quick-firing guns, which is near the melting point of the raw material. This has the result that a measurable quantity of fused or vaporized material leaves the barrel with the projectile during firing. Insofar as such material comes from the driving band of the projectiles, no drawbacks need be anticipated. But if the material ejected stems from the inner barrel wall, this definitely involves a highly undesirable wear of the barrel, at any rate where the material has been removed. Weighing of the barrels of quick-firing guns prior and subsequent to firing revealed weight losses of up to 100 gms.

In order to improve the life of the heavy-duty barrels of firearms, such barrels have their inner wall improved,

preferably by nitriding according to Swiss Patent No. 308,295.

It has been found that tests performed with projectiles previously subjected to various treatments resulted in a reduction of the quantity of material removed from the inner barrel wall by melting. Such a reduction of wear was always noticed when the melting point of the material of the driving band was at least substantially reduced so as to approach the melting point of the inner barrel wall or lowered beneath that value. Apparently a certain quantity of fused and vaporized material is necessary for the passage of the projectiles through such firearm barrels; if the melting point of at least the projectile driving bands is lower than the melting point of the inner barrel wall, the fused material is largely supplied by these projectile portions and not by the inner barrel wall. This protection of the inner barrel wall would appear to have caused the noticed improvement of the resistance to wear and of the life.

Naturally it is not necessary that the melting point of the projectile driving bands be reduced exactly to the melting point of the surface portions of the inner barrel wall since an approximate adjustment suffices to result in a marked improvement of the life. By way of example, compared with projectiles without nitrided steel driving bands, a substantial prolongation of the life of gun barrels of which the inner walls had been nitrided according to the method disclosed in Swiss Patent No. 308,295 was obtained when steel projectiles having nitrided steel driving bands were used.

It is particularly advantageous to adjust the melting point of the projectile driving bands to the melting point of the inner barrel wall by forming at least the said bands of a steel of which the melting point has been lowered by diffusing suitable foreign substances into it. By way of example, if the steel driving bands of steel projectiles are to be annealed and simultaneously enriched with nitrogen, an arrangement according to FIG. 1 can be employed. To this end, an evacuable double-walled and coolable gas-discharge vessel 1 with a removable lid 2 has its interior provided with a metallic supporting plate 3 on insulators 4 carrying resilient metal pins 5 designed to have the steel projectiles 6 slipped over them. Arranged parallel with the supporting plate 3 and conductively connected therewith is a metallic orifice plate 7 arranged in a plane with the driving bands 8 of the projectiles 6 and provided with circular holes 9 through which the projectiles 6 project. The thickness of the orifice plate 7 is such as to cause the inner side of the holes 9 to register with the two driving bands 8. This inner side of the holes 9 must enclose the driving bands 8 concentrically and form an annular gap with them which is of the same width throughout.

The supporting plate 3 and the orifice plate 7 are connected with the negative pole of the pair of terminals 11 via an insulated voltage lead-in 10, while the positive connection is effected with the metallic discharge vessel 1. In the discharge vessel 1, 2, suitable means (not shown) are provided to produce a gas atmosphere comprising 30% N<sub>2</sub> and 70% H<sub>2</sub> at a pressure of 5 to 10 mm. Hg, and to maintain it during operation. After completion of a starting cycle, a glow discharge is produced at a voltage of 400 to 500 volts between the discharge vessel 1 and the projectiles 6 and on the orifice plate 7 connected to the same voltage. This glow discharge produces a particularly elevated energy concentration of .1 to 10 watts/cm.<sup>2</sup> of the surface of the driving bands 8 between the said bands and the inner wall of the holes 9 if the width of the annular gap is suitable. This operative condition, which is termed hollow-cathode effect, is described in detail in the Swiss Patent No. 314,340. The driving bands 8 reach the desired glow temperature during this type of operation

within a short space of time, e.g. .5 to 2 minutes, and are enriched with nitrogen owing to the ion bombardment. The high energy density in the annular gap ensures a comparatively rapid diffusion of the atomic nitrogen into the driving bands so that the necessary penetration depth is obtained after annealing, and the treatment can be discontinued. Within the relatively short period of treatment the projectile 6 has the temperature of its other portions increased so slightly only that its strength is not affected.

When the treatment gases are diffused into the metal surface, i.e. the nitrogen in the example disclosed above, so called solid solutions are formed which constitute chemical and physical combinations of metal and gas. Experience has shown that such solid solutions—also under the extreme pressure conditions during firing—result in a reduction of the melting point of the steel driving bands to a value which corresponds approximately to the melting point of the inner wall of gun barrels nitrided according to the above-mentioned Swiss Patent No. 314,340.

Apart from the above-mentioned nitrogen and according to the application, many other substances are suitable. By way of example, the projectile portions can be enriched with phosphorus or with sulphur, either in elementary form, dissolved in the metal involved, as solid solution, or in the form of suitable compounds.

Finally, other gases, such as hydrogen, oxygen and—under certain conditions—even rare gases may be concentrated in the projectile portions in question in such a form that they can contribute to reducing the melting point.

As in the example described above, the substances to be concentrated in the projectile driving bands may be obtained mainly from the gas in the discharge vessel. Naturally such foreign substances may also be applied in some other manner to the projectile surfaces to be treated in the glow discharge.

By way of example, a suitable substance may be vaporized in the discharge vessel and mixed with the gas atmosphere, or a corresponding mist formed of such material particles is sprayed into the discharge vessel. In addition, the known process of cathode atomization or arc dusting may be employed to mix the foreign particles with the gas atmosphere.

The present method is of course not limited to the treatment of projectiles which have at least the driving bands adjusted to the gun barrel by means of an electric gas or glow discharge and by enrichment with foreign substances. Enrichment with foreign substances may also be obtained in some other manner, by way of example by diffusion in heatable furnaces or by treatment in melts containing the said foreign substances. It is also possible to form the projectiles or at least their driving bands of materials of which the melting point is already adjusted to that of the associated gun barrel without additional treatment.

The improvement of the life of gun barrels performed in the manner disclosed and the present method of treating projectile driving bands is probably also the result of the simultaneous formation of a gaseous slide film on the surfaces in engagement. It has been known for some time that a gas layer between the metal surfaces of firearm barrels and projectiles sliding on one another at a high pressure per unit area can substantially reduce friction. The gaseous lubricant film is not supplied to the contacting surfaces from outside but provided by vaporization of gas-generating materials from the surfaces in engagement or the issuance of gas components dissolved in the metal or combined with the metal surface, which is naturally possible only under high surface pressure. Naturally normal unprepared sliding surfaces cannot maintain a gaseous lubricant film for any length of time since a certain gas loss by diffusion into the as-

sociated surface and by the passage towards the edges of the sliding surface portions is inevitable.

It has therefore been proposed to increase the gas supply by the surfaces subject to sliding friction of the barrel and projectile respectively by charging their surfaces with gases or by diffusing gas generating substances into them. Phosphorus, sulphur, certain metals, oxygen etc. are suitable materials. It has also been proposed to design the driving bands of the projectiles correspondingly and to enrich them with gas generating substances, i.e. to charge them with gas at the surface, instead of treating the inner wall of the gun barrels, which are difficult to process. Attempts at obtaining a further reduction of sliding friction by influencing the degree of enrichment in the metal surfaces involved (distribution of depth, concentration etc.) have been unsuccessful and revealed only a slight influence on the maximum reduction of friction.

It was astonishing to find a further improvement of the life of firearm barrels after lowering the melting point according to the present method, if a material component is provided at least in the projectile driving bands which release that foreign substance under the conditions obtaining during firing which has been concentrated in the inner surface of the barrel.

In the gun barrels having their inner wall enriched with nitrogen by an electric glow discharge, the surface portions engaged by the projectile can easily supply the quantity of gas required for the formation of gas pads. During the passage of standard projectiles provided with unprepared driving bands it would seem that a certain quantity of gas is used and thus results in a detrimental reduction of the gaseous lubricant film.

Conditions are somewhat different with the application of gas nitrided projectile driving bands, which has already been experimentally attempted at an earlier date, in standard, i.e. not specially prepared, gun barrels. The driving bands nitrided in conventional baths or furnaces could, however, supply a friction-reducing gas pad while the barrels were still cold, but during rapid fire this advantageous gas layer could not be maintained. Apparently the heated inner barrel wall absorbs the gases emerging from the driving bands far too rapidly for a gaseous lubricant film to be maintained.

With the present method, both the gun barrels and the driving bands of the projectiles which will contact their inner walls are enriched with suitable substances, e.g. in an electric glow discharge.

The tests made in this connection revealed a further improvement of the life of firearm barrels beyond the values previously obtained if a material component was provided in the projectile driving bands which will release that foreign substance in firing with which the inner wall of the barrel has been enriched. The gas layer formed when the high sliding friction occurs is no longer supplied by the inner barrel wall as hitherto and more or less absorbed by the driving bands. The driving bands contribute to the supply of the gas layer. If the driving bands become heated during their passage through the barrel when single rounds are fired, the reduction of gas generating substances in the inner barrel wall is largely prevented since just those substances are supplied by the driving bands and partly diffused into the heated inner barrel wall with which the latter has been enriched and improved.

Both surfaces are preferably enriched with the same gas generating substance. However, different substances may be employed provided that the projectile driving bands supply those gaseous components with which the inner barrel wall has already been enriched.

Furthermore, it is important that the concentration of the gas generating substances enriched in the two metal surfaces are adapted to one another. As gun barrels must advantageously be nitrided in an electric gas or glow discharge in order to obtain a hardened but ductile and

shatterproof inner surface, it is recommended to enrich the entire outside of the projectile, or at least the projectile portions designed to contact the said inner wall, in an ionized gas atmosphere with the same gas generating substances although the present method is not limited to this treatment of the projectiles.

The gas generating substances can either enrich, as chemical compounds, the topmost zones of the projectile driving bands, or form alloy components of the metals employed or a solid solution with the metal. Apart from such chemical compounds, metals and metalloids are suitable as alloy components when concentrated in the inner barrel wall, by way of example zinc, lead, chromium etc. In all cases, the desired reduction of the melting point is obtained as well.

In the treatment disclosed in conjunction with the drawing, of metal surfaces in a glow discharge, the surface structure by material migration caused by dissolving minute metal particles from the surface zone is altered also when the said surfaces are not heated to annealing temperature as in the above example. It is not exactly known whether the metal particles are dissolved out of the crystal structure owing to vaporization at the points of impingement of individual ions or owing to direct shock release. At any rate, experiments reveal migration of the material. At the same time material is also added since the gas atmosphere is intermingled with metal particles stemming from the surface of the work itself or from the counter-electrode, and such metal particles are electrically charged in the glow chamber, accelerated in the direction of the work surface and impinge on the latter with a high kinetic energy.

The extent of the material migration in one or the other direction can be influenced by suitable selection of the geometric arrangement of the work and the counter-electrode as well as by the pressure in the discharge vessel and the type and polarity of the voltage. The conditions of the discharge are advantageously so selected that material removal is preponderant. At any rate, the surface of the work is provided, after maintaining the glow discharge for a sufficient space of time, which is only a few minutes in the example described, but may be hours, with a surface zone on the metal body which displays a highly uniform micro-porosity, which is likely to extend into molecular dimensions. At the same time, this surface zone has a strength not markedly inferior to that of unaltered metal layers.

This micro-porous surface layer keenly enriches itself with the gas present in the discharge vessel and retains this gas charge also after completion of the treatment and under atmospheric conditions.

After this glow-discharge treatment, the surface is enriched with gas in two respects. On the one hand, nitrogen diffused into it is dissolved in the metal layer or combined in the form of a solid solution. On the other hand, gaseous components are enclosed or adsorbed in the micro-porous surface layer. Under the pressure and temperature conditions prevailing in firing, both the gas charge and the solid solutions contribute to the supply of the friction-reducing gas layer between the metal surfaces sliding on one another. As regards the driving bands, the gas charge is likely to be effective at the outset while substantially deeper zones having solid solutions contribute to the supply of gas after deformation has begun.

Depending on the foreign substances concentrated in the inner barrel wall and apart from the above-mentioned solid nitrogen-metal solutions, many other substances are

suitable to supply gas. By way of example, the projectile portions can be enriched with sulphur either in elementary form, dissolved in the metal involved as a solid solution, or in the form of suitable compounds.

5 Such substances evaporate under the extreme pressures and temperatures prevailing and form the friction-reducing gas layer. Finally, other gases, such as hydrogen, oxygen and—under certain conditions—rare gases may be concentrated in the metal surfaces subject to friction so that they may contribute to the formation of friction-reducing gas layers in order to avoid a reduction of the said substances in the inner barrel wall.

It may also be pointed out that the friction-reducing gas pad is advantageous for firearms owing to the efficient sealing of the projectile in the barrel. The pressure-reducing gas layer obtained also seems to form a protective layer for the portions of the inner barrel wall subject to particular stress against the aggressive explosion products.

10 It may be possible that the marked improvement of the life of firearm barrels obtainable by means of this method is not caused by the reduction of the losses due to sliding friction itself, but to the reduction of detrimental effects of the usually high sliding friction, such as wear, increased danger of erosion etc.

25 I claim:

1. Method of reducing wear of the inner wall of a steel gun barrel, hardened by nitriding, by the passage therethrough of projectiles on firing, the driving bands of the projectile being made of a ferrous material having a 30 higher melting point than the hardened barrel inner wall, comprising heating the projectile driving bands in a medium containing a substance which diffuses into the surface zones of the projectile driving bands which later, on firing, slide along the barrel inner wall and are capable of developing and releasing gases or vapors at the 35 temperature occurring on firing which build up a friction-reducing film between the barrel wall and the driving bands, and continuing the treatment to cause said substance to diffuse into the driving bands in such amount that the melting point of the surface zones of the driving bands, enriched with such substance, is reduced down to or below the melting point of the hardened surface zone of the barrel inner wall.

2. Process according to claim 1, wherein the medium 45 in which the driving bands are heated is a gaseous or vaporous atmosphere containing the said substance.

3. Process according to claim 2, in which the driving bands are heated by an electric glow discharge in the said atmosphere.

40 4. Process according to claim 1, wherein the medium in which the driving bands are heated comprises an atmosphere containing nitrogen.

5. Process according to claim 1, wherein the driving bands to be treated possess a microporous surface zone.

55

#### References Cited in the file of this patent

#### UNITED STATES PATENTS

|           |          |               |
|-----------|----------|---------------|
| 1,837,256 | Egan     | Dec. 22, 1931 |
| 1,861,522 | Brandt   | June 7, 1932  |
| 2,411,073 | Whitney  | Nov. 12, 1946 |
| 2,437,249 | Floe     | Mar. 7, 1948  |
| 2,701,524 | Van Dine | Feb. 8, 1955  |

65

|         |               |               |
|---------|---------------|---------------|
| 589,069 | Great Britain | June 10, 1947 |
| 744,753 | Great Britain | Feb. 15, 1956 |

#### FOREIGN PATENTS